

July 31, 1945.

I. E. BERKOVITS

2,380,718

MANUFACTURE OF PAPER FOR STENCIL SHEETS

Filed Nov. 28, 1940

Fig.1



Fig. 2



INVENTOR.

*Isaac E. Berkovits*

Patented July 31, 1945

2,380,718

# UNITED STATES PATENT OFFICE

2,380,718

## MANUFACTURE OF PAPER FOR STENCIL SHEETS

Irene Elisabeth Berkovits, New York, N. Y.

Application November 28, 1946, Serial No. 367,535

12 Claims. (Cl. 101—128.2)

This invention relates to the manufacture of long fibre paper suitable for the production of stencil sheets as used in the art of duplicating or mimeographing.

Conventional stencil sheets consist of paper made impervious to ink by suitable impregnation or coating. When an impression is effected on the sheet by the type of a typewriter or a stylus, the sheet is made pervious to ink along desired lines to form an outline for the character or drawing to be reproduced. In this operation it is essential that the material of the sheet consists of long fibres of sufficient strength to prevent the type of the typewriter or the stylus from cutting out the centers of loop letters or the like so that distortion of the outlines is avoided. After the necessary impressions have been made, one face of the stencil sheet is coated with ink which will pass through the sheet along the desired lines only, so that a true reproduction may be obtained on a sheet of paper brought into contact with the other face of the stencil sheet.

In the past, stencil sheets of the above character have been produced from special long fibre Japanese paper, the so called "Tosa Tengujo" paper which has the required strength. Various attempts have been made to replace this paper by other products, but these substitutes have not been satisfactory for use in the stencil paper industry.

One object of the present invention is to provide long fibre paper which is made of readily available raw material at low cost and is equivalent or superior to Japanese paper regarding its qualities.

Another object of the invention is to provide a method of manufacturing long fibre paper for stencil sheets, in which a thin carded web of cotton or other downy or fluffy fibrous material of the type commonly employed in the textile industry as raw material is used as the starting material for making the long fibre paper.

A further object of the invention is to provide a simple and efficient apparatus for the manufacture of paper for stencil sheets.

It is also an object of the invention to provide a stencil sheet for duplicating or mimeographing purposes, which does not have an oily appearance.

Other objects and advantages will become apparent as the description proceeds.

For the purpose of illustration, but in no sense of limitation, certain preferred embodiments of the invention will be described hereinafter with reference to the accompanying drawing.

In the drawing,

Fig. 1 is a diagrammatic elevational view showing an apparatus for carrying out the invention.

Fig. 2 is a similar view showing a modified apparatus which operates substantially automatically.

In carrying out the invention, a web of cotton obtained from comberwaste by carding is preferably used as the starting material. Such carded web of cotton weighs approximately 12 to 16 g./m.<sup>2</sup> and has heretofore been employed in the textile industry as a raw material. However, a carded web of downy or fluffy fibrous textile material other than cotton may also be used, for example, a carded web of wool, silk, or the like.

When the apparatus shown in Fig. 1 is employed, the carded web is first cut at a cutting station (not shown) into blanks *a* of a length and width corresponding substantially to the size of the desired stencil sheets. The cutting is preferably performed in such manner that the fibres of the web material extend in the longitudinal direction of the blanks. Each blank *a* is then supported by a member *b* of felt or the like which may be somewhat larger than the blank member, and both the blank and the felt are placed on a conveying belt *f* to be advanced through a chamber *2* in which the blank is impregnated with an adhesive. The adhesive substance may be sprayed upon the blank and is supplied to chamber *2* in the direction of the arrow indicated at the upper end of the chamber.

The impregnation may be carried out with any well known stiffening and adhesive substance or sizing material such as natural or synthetic resin, glue, starch casein, varnish, etc.

The impregnated blank is placed on a table *4* and covered with a felt member *c* similar to member *b*. The blank *a* and felt members *b*, *c* are then passed between a pair of rolls *3* heated to a temperature approximately 50° to 60° C. The felt members protect the blank during this initial drying step and may also absorb excess liquid.

On the table *5* the blanks are removed from between the felt members and then placed on the conveying wire *6* to be advanced through the drying chamber *7*. The dry blanks are compressed in a hydraulic press (not shown), in which a plurality of sheets are preferably treated at the same time, and they are then ready for use as paper blanks for the production of stencil sheets.

When producing such stencil sheets, the paper blanks will be impregnated or coated with a substance impervious to ink. While such final impregnation usually renders Japanese stencil paper oily, it is an additional advantage of the improved

material according to the present invention that due to its high absorbing capacity it is not of such oily appearance so that it is easier to handle.

Referring now to Fig. 2, the apparatus illustrated therein performs most of the necessary steps automatically. In the method carried out on this apparatus, a carded web *d* is used which is disposed between protective paper layers *e*, *j*. The carded web and protective layers are provided in coil form on a reel *8* from which they are unwound, the protective layers being received by the winding reels *9*, *10*, while the web is advanced by means of a conveyor *11*. The endless flexible member *g* of this conveyor consists of felt or the like and one or both of the conveyor rolls may be heated to dry the felt member. The conveyor *11* will pass web *d* through the impregnating chamber *2* identical with or similar to chamber *2* shown in Fig. 1, and through a pair of heated rollers *3'* which correspond to rollers *3* of Fig. 1. In the embodiment according to Fig. 2, an endless felt member *h* passing over guide rolls *12*, *13*, *14* is arranged to cover the upper face of web *d* while the web travels through rollers *3'*. One or more of the guide rolls *12*, *13*, *14* may be heated to dry felt member *h*.

When leaving the conveyor *11*, the web is passed through a suitable guide *15* into a drying chamber *16* having a conveyor *17*. Thereafter, the dry web is advanced by a conveyor *18* to cutting station *19* where it is cut into paper blanks of proper dimensions. The blanks are compressed in a hydraulic press in the manner described in connection with Fig. 1 and are ready for use in stencil sheet production in which they will receive an impregnation or coating by a substance impervious to ink.

One particular advantage of the invention resides in the use of a starting material which is readily available. Moreover, the long fibre paper obtained by the method of the invention is considerably cheaper than the "Tossa Tengujo" paper used at present in the stencil paper industry.

While certain preferred embodiments of the invention have been described hereinabove and illustrated in the accompanying drawing, it is to be understood that the invention is not limited to the precise details so illustrated and described, but that various changes may be resorted to without departing from the scope of the appended claims.

What is claimed is:

1. Thin fibrous sheet material adapted for conversion into stencil sheet by incorporation therewith of ink-impervious material capable of being rendered locally ink-permeable by stylus impressions, consisting of a thin, flatwise compact sheet of carded, predominantly parallel, long cotton fibers, said fibers being provided with adhesive material comprising paper size securing them together and constituting an ink-permeable, compressed, paper-thin sheet.

2. A compressed, carded cotton sheet of substantially long cotton fibers in carded form and adhesively secured together with paper size, said adhesively secured fibers being in thin, compressed form and thereby constituting an ink-permeable, paper-like sheet adapted for use as a base in a stencil sheet.

3. A stencil sheet comprising a thin sheet base of compressed, predominantly parallel, substantially long cotton fibers in carded form, said fibers being adhesively secured together with paper size and said base sheet carrying a coating of ink-impervious material penetrable by stylus impres-

sions, and thereby providing a stencil sheet of normally ink-impervious character adapted to be rendered locally ink-permeable by stylus impressions.

4. A stencil sheet comprising a thin, flat-wise compressed sheet of carded, substantially long cotton fibers having incorporated therewith paper size and a coextending film of ink-impervious material susceptible of displacement by stylus impressions and thereby providing, with said carded cotton sheet, a thin, normally ink-impervious stencil sheet adapted to be rendered locally ink-permeable by stylus impressions.

5. A stencil sheet comprising a thin, compressed, ink-permeable, paper-like sheet of adhesively cohering carded cotton fibers of the character used for making textiles, said thin, carded fiber sheet having incorporated therewith a coextending, normally ink-impervious but stylus-penetrable film.

6. A stencil sheet comprising a thin, compressed sheet of carded cotton fibers of the character used for making textiles, said fibers being sized to constitute a coherent sheet and being predominantly disposed in parallel relation to each other, and said cotton sheet carrying a coating of ink-impervious material rendering said sheet normally impervious to the ink, but capable of being made locally permeable to ink by stylus impressions.

7. A method of manufacturing a base material for stencil sheets, comprising forming a thin web of substantially long cotton fibers of the character used for making textiles and applying adhesive material to said web and compressing the web to provide a thin, ink-permeable cotton fiber sheet adapted to be converted into a stencil sheet by application of ink-impervious material, said adhesive applying and sheet-compressing procedure including applying liquid adhesive material containing proper size throughout the cotton fiber web and drying the web, to effect adherence of the fibers together while maintaining ink-permeability thereof, and compacting the web by substantially high pressure flat-wise thereof.

8. A method of manufacturing a base material for stencil sheets, comprising forming a thin web of carded, substantially long cotton fibers, and applying adhesive material to said web and compressing the web to provide a thin, ink-permeable cotton fiber sheet adapted to be converted into a stencil sheet by application of ink-impervious material, said adhesive applying and sheet-compressing procedure including applying liquid adhesive material containing paper size to the cotton fiber web, compressing the web while maintaining the same in contact with absorbent surfaces on opposite sides, drying the web and compacting the same by substantially high pressure flat-wise thereof.

9. A method of manufacturing stencil sheets, comprising forming a thin web of carded, substantially long cotton fibers, and converting said web into a stencil sheet by procedure including sizing the web, compressing the web flat-wise and applying thereto a co-extending film of ink-impervious, stylus-penetrable material.

10. A method of manufacturing stencil sheets, comprising forming a thin, ink-permeable web of carded cotton fibers of the character used for making textiles, applying adhesive material to said web and drying and compressing the same to convert the web into a thin sheet of adhesively-secured cotton fibers while maintaining the sheet in ink-permeable form, and converting said sheet

to a stencil sheet by applying an ink-impervious, stylus-penetrable coating material thereto.

11. A method of manufacturing stencil sheets, comprising forming a thin web of substantially long cotton fibers of the character used for making textiles, converting said web into a thin, coherent, ink-permeable cotton fiber sheet by procedure including applying adhesive material containing paper size throughout the web and compressing the same, and converting said cotton fiber sheet into a stencil sheet by impregnating said cotton fiber sheet with ink-impervious, stylus-penetrable material.

12. A method of manufacturing stencil sheets, comprising forming a thin web of carded, substantially long cotton fibers, applying adhesive

material to said web and compressing the web to provide a thin, ink-permeable cotton fiber sheet adapted to be converted into a stencil sheet by application of ink-impervious material, said adhesive applying and sheet-compressing procedure including applying liquid adhesive material containing paper size throughout the cotton fiber web, compressing the web while maintaining the same in contact with absorbent surfaces on opposite sides, drying the web and compacting the same by substantially high pressure flat-wise thereof, and converting said cotton fiber sheet into a stencil sheet by applying to said cotton fiber sheet a coextending film of ink-impervious, stylus-penetrable material.

IRENE ELISABETH BERKOVITS.